

Patented Aug. 24, 1926.

1,597,189

# UNITED STATES PATENT OFFICE.

WILLIAM BENJAMIN GERO, OF EAST ORANGE, NEW JERSEY, ASSIGNOR, BY MESNE ASSIGNMENTS, TO WESTINGHOUSE LAMP COMPANY, A CORPORATION OF PENNSYLVANIA.

## METHOD OF COLD-DRAWING REFRACORY MATERIALS.

No Drawing.

Application filed January 11, 1921. Serial No. 436,597.

This invention relates to the art of wire drawing and particularly to the cold drawing of refractory metals.

It has for one of its objects the provision of a more economical and efficient method of drawing such metals and is especially applicable to the cold drawing of molybdenum.

Another object of the invention is the provision of a method for drawing said metals which will yield a product of higher tensile strength and resilience and in general possess better qualities as a support for a filament in incandescent lamps than could be secured heretofore.

15 A special object is the provision of a copper-coated molybdenum wire for use in incandescent lamps.

According to the best process heretofore known, molybdenum wire was drawn hot to about 20 mil diameter, because of the extreme difficulty of drawing it cold. However, to secure the valuable effects of cold working, it was necessary to draw the molybdenum cold from about 20 mil diameter to finished sizes. In the process of cold drawing, the wire became so hard that, coming in contact with the die, an excessively high rate of die wear resulted. It was, therefore, necessary to anneal the wire frequently in order to soften it. The annealing process, however, caused the wire to lose the desirable properties which had been given it by the cold working.

While an adherent coating of a lubricant, such as graphite, could be baked on in a hot drawing process, this could not be done with small-size wire because the temperature necessary to accomplish this would weaken such small wire sufficiently to make it impractical to draw it. The small-size wire, therefore, had to be cold drawn without a lubricant.

Another disadvantage of former processes was the gradual increase in diameter of a single piece of wire as it was drawn through the die on account of the high rate of die wear. The frequent breaking of the wire necessitated the use of a single-head wire-drawing machine instead of the much more efficient multiple-head type of machine, thereby causing the efficiency of the machine and of the operator to be low.

My invention provides a process whereby a refractory metal may be worked cold to

any extent without the necessity of annealing. Since the amount of cold working which a metal receives determines the degree of certain of its physical properties, my invention provides a method of controlling the degree of these properties within certain limits.

It is a well-known fact that the cold working of the metal hardens it and gives it a higher tensile strength and greater resilience, and that the process of annealing produces opposite effects. A metal which has been worked while cold often possesses valuable properties in a higher degree than is possessed by the same metal when worked hot; for instance, cold working gives a metal of greater hardness and higher tensile strength than does hot working.

This invention provides a process for cold working refractory metals which heretofore have had to be worked hot because of the lack of a process by which they could be worked cold.

In drawing soft metal into wire there is practically no wear on the dies. By coating a hard metal, such as molybdenum, with a soft metal, thus interposing a layer of soft metal between the hard molybdenum and the die, the hard metal can be drawn with the die wear of the soft metal. The soft metal acts as a lubricant for the drawing of the hard metal. The advantage in using a metal coating as a lubricant instead of graphite or greases lies in the fact that the metal provides a continuous coating, whereas other lubricants are more or less discontinuous or non-uniform so that they allow the wire to touch the die at some points.

Although soft metals have heretofore been proposed as lubricants, they seem to have proved unsatisfactory in drawing refractory metals because of the great difficulty experienced in applying them to the metal to be drawn. Apparently, they could not be made to adhere to a body composed of refractory metal.

100 In practicing my invention, a molybdenum wire or rod is coated with copper or other soft metal which will serve as a lubricant. Brass, lead and other soft alloys and metals have been successfully used as lubricants. 105 For the purpose of describing my invention, copper will be taken as the representative metal for encasing the molybdenum. I pre-

fer to copper plate the molybdenum by applying a coating of copper oxide, reducing the oxide and melting the copper. The body of molybdenum, which may be a rod, is coated by passing it through a mixture which consists of copper oxide suspended in an alcoholic solution of shellac. This mixture may consist of 100 cc. of an 18% alcoholic solution of shellac and 100 grams of 200 10 mesh copper oxide; the proportions may be varied to suit varying conditions, such as the amount of reduction to be made in the diameter of the rod and the thickness of the copper coating desired in the product. The 15 coated rod is then passed through an electric furnace having a reducing atmosphere, such as hydrogen, and a temperature somewhat above the melting point of copper, the temperature depending on the rate at which 20 the wire is passed through the furnace. The copper oxide is thereby reduced to copper and the latter fused to the wire in a smooth coating which will adhere to the molybdenum through swaging, rolling, drawing, and 25 other ordinary operations used in its fabrication. This method of applying the copper produces a copper coating of the desired softness. Using an additional lubricant, such as a soap solution, the copper coated 30 molybdenum wire is drawn cold, which may now be done on a multiple-head wire-drawing machine, to any desired diameter without the necessity of annealing. The copper remains as a sheath on the molybdenum core 35 to the smallest gage desired. The copper-coating may then be dissolved off or retained as desired.

If the copper-coated molybdenum is used as a support for a tungsten filament of an incandescent lamp, part of the copper is oxidized to copper oxide by a flame used during the operation of inserting the support into the button of the arbor of the lamp. This 40 copper oxide acts as a getter or beneficial agent to improve the quality of the lamp.

By means of this invention, allowing refractory metals to be cold worked, the finished product possesses improved physical properties which could not be secured by 45 previous processes of working, thereby making it more valuable for various uses, especially as a support for a filament of an incandescent lamp.

Another improvement in the art which 50 this invention provides is a process by which certain physical properties of a metal may be regulated within a certain range. This is accomplished because my invention permits any amount of cold working to be done on 55 the metal, and because the amount of cold working determines the degree of certain physical properties.

The superior qualities possessed by wire 60 manufactured according to the present invention allow the use of wire of smaller di-

ameter for a given purpose than is necessary with hot-drawn wire or with wire which has been annealed, whereby a considerable economy is effected in the use of expensive metals.

What is claimed is:

1. The method of cold-working a refractory metal of the groups including molybdenum, tantalum, tungsten, chromium, zirconium, uranium, thorium and the like, which comprises coating the metal with a continuous sheath of a metallic material to serve as a lubricant and cold-working the coated metal.

2. The method of cold-working a refractory metal of the groups including molybdenum, tantalum, tungsten, chromium, zirconium, uranium, thorium and the like, which comprises fusing upon said metal a coating of a metallic material which serves as a lubricant and cold-working the coated metal.

3. The method of cold-drawing a refractory metal of the groups including molybdenum, tantalum, tungsten, chromium, zirconium, uranium, thorium and the like, which comprises coating said metal with a reducible compound of a metal which has a lubricating property, reducing the said oxide to its metal, fusing the metallic coating and cold-drawing the coated metal.

4. The method of cold-working a refractory metal of the groups including molybdenum, tantalum, tungsten, chromium, zirconium, uranium, thorium and the like, which comprises coating said metal with a metallic oxide reducible by hydrogen, the metal of which has a lubricating property, reducing the said oxide to its metal, fusing the metallic coating and cold-working the coated metal.

5. The method of working molybdenum, which consists in coating it with a continuous sheath of a metallic lubricating material and working the metal-coated molybdenum cold.

6. The method of drawing molybdenum, which consists in coating a molybdenum rod with a continuous sheath of a metallic lubricating material and then cold-drawing the coated rod.

7. The process of drawing molybdenum which consists in coating said metal with a reducible oxide of a metal which has a lubricating property, reducing the said oxide to its metal, fusing the metallic coating, and cold drawing the metal-coated molybdenum.

8. The process of working molybdenum which consists in coating said metal with a metallic oxide reducible by hydrogen, the metal of which has a lubricating property, reducing the said oxide to its metal, fusing the metallic coating and cold-drawing the metal-coated molybdenum.

9. The process of working molybdenum which consists in coating said metal with copper oxide, reducing said oxide to copper,

fusing the copper and cold working the copper-coated molybdenum.

10. As an article of manufacture, a body of refractory metal of the groups including molybdenum, tantalum, tungsten, chromium, zirconium, uranium, thorium and the like clad with an adherent fused coating of copper reduced from the oxide thereof while the latter is on said metal.
11. As an article of manufacture, a body of refractory metal of the groups including molybdenum, tantalum, tungsten, chromium, zirconium, uranium, thorium and the like clad with an adherent coating of copper sintered to said refractory metal by reducing an oxide of copper in the form of a coating on said refractory metal.
12. As an article of manufacture, a body of molybdenum coated with an adherent metal formed by reducing an oxide of the latter on said molybdenum.
13. As an article of manufacture, a body of molybdenum clad with a coating of copper united to said molybdenum by reducing an oxide of copper thereon.
14. A resilient support for the filament of an incandescent lamp consisting of a copper-coated molybdenum wire formed by reducing an oxide of copper on said molybdenum wire.
15. As an article of manufacture, a composite body comprising a refractory metal of the groups including molybdenum, tantalum, tungsten, chromium, zirconium, uranium, thorium and the like, coated with a fused coating of a metal, the oxide of which is reducible, said coated refractory metal capable of being worked without material alteration in the relative proportions of the coating material and the refractory metal.
16. As an article of manufacture, a composite body comprising a refractory metal of the groups including molybdenum, tantalum, tungsten, chromium, zirconium, uranium, thorium and the like, clad with a fused coating of copper, said clad body capable of being worked without material alteration in the relative proportions of the copper and refractory metal.
17. As an article of manufacture, a mechanically worked metallic core of a refractory metal having formed thereon by the reduction of an oxide of copper, an adherent fused coating of copper.
18. As an article of manufacture, a cold worked metal having an integral coating of copper formed thereon by reducing the oxide of copper.

In testimony whereof, I have hereunto subscribed my name this tenth day of January 1921.

WILLIAM BENJAMIN GERO.